

May 11, 1926.

1,583,788

A. G. GILMAN

# METHOD OF AND APPARATUS FOR FINISHING PAPER

Filed Oct. 20, 1924

2 Sheets-Sheet 1



BY Alexander G. Gilman  
Chappell & Ward  
ATTORNEYS

May 11, 1926.

A. G. GILMAN

1,583,788

METHOD OF AND APPARATUS FOR FINISHING PAPER

Filed Oct. 20, 1924

2 Sheets-Sheet 2



FIG. II.

INVENTOR  
Alexander G. Gilman  
BY  
*Chappell & Carl*  
ATTORNEYS

## UNITED STATES PATENT OFFICE.

ALEXANDER G. GILMAN, OF KALAMAZOO, MICHIGAN.

## METHOD OF AND APPARATUS FOR FINISHING PAPER.

Application filed October 20, 1924. Serial No. 744,737.

This invention relates to improvements in a method and apparatus for finishing paper.

The main object of this invention is to provide an improved method of finishing 5 coated paper whereby a uniformly smooth even surface and texture is secured.

A further object is to provide a method of finishing paper by which the above results may be secured with a minimum of coating.

10 A still further object is to provide an apparatus for finishing coated paper securing the above results which is of large capacity and at the same time very compact.

Objects relating to details and economies 15 of construction and operation will definitely appear from the detailed description to follow.

I accomplish the objects of my invention by the devices and means described in the 20 following specification. The invention is clearly defined and pointed out in the claims.

A structure which is a preferred embodiment of my invention is clearly illustrated in the accompanying drawing, forming a 25 part of this application, in which:

Fig. I is a diagrammatic view of an apparatus for finishing paper by my improved method.

Fig. II is a fragmentary perspective view 30 of one of the units employed in the finishing of paper by my improved method.

In the drawing similar reference characters refer to similar parts throughout the several views.

35 Referring to the drawing, I have diagrammatically illustrated in Fig. I the units employed by me in the complete finishing of paper by my improved method. This consists of a coating machine designated generally by the numeral 1, the particular machine illustrated being designed to apply a coating to one side only of the paper.

From the coating machine the paper is 40 passed to a drier, indicated generally by the numeral 2, this drier being of the loop type and also being shown conventionally. The passage of the paper through the drier is designed so that when the paper is delivered therefrom, the coating approximates but 45 has not reached the setting point.

From the drier the paper is passed 50 through a smoothing machine which consists of a supporting cylinder 3, a plurality of guide rollers 4 and 5 and polishing or smoothing brushes 6 which are disposed to

coact upon the web of paper 7 while it is supported by the cylinder 3.

The brushes 6 act upon the coated surface of the paper, brushing and smoothing the partially dried coating and forcing the same 60 into the pores of the paper. These brushes are of fine material, that is, they have relatively fine filaments, the filaments being thickly set and forming quite a firm compact body. In practice, the brushes 6 are driven at a relatively high rate of speed so that as the paper passes over the cylinder the coating is subjected to a very substantial brushing and smoothing action. The coating, however, is sufficiently dried while subjected to this action so that no material amount is removed by this treatment.

From the polishing or smoothing machine, the paper is passed to a roll 8, or to a calendering machine indicated 70 conventionally at 9, the calendering machine being employed when it is desired to provide the paper with a high polish. A satisfactory coating is that commonly designated as "enamel" coating, commonly consisting of china clay, casein and satin white, the proportions being varied according to the grade of enamel. The satin white is entirely omitted in certain low grade enamels, the percentage increasing in the higher 85 grades as will be readily understood by those skilled in this paper coating art.

By my improved finishing method, I am enabled to produce a uniform finish of a very fine smooth character and this may be 90 accomplished with a minimum of coating.

While the units employed by me in practicing my improved method of finishing paper are mainly shown in conventional form, it is believed the disclosure made will enable those skilled in the art to which my invention relates to embody or carry out my invention as may be best suited or most practical for the particular mill or installation.

Having thus described my invention, what I claim as new and desire to secure by Letters Patent, is:

1. The method of finishing paper consisting of coating with an enamel coating, passing through a drier to dry to approximately the setting point of the coating, subjecting while in such condition of dryness to the action of a rotating brush, and calendering.

2. The method of finishing paper consist-

ing of coating with an enamel coating, passing through a drier, subjecting while in approximately dry condition to a brushing action, and calendering.

5. An apparatus for finishing paper comprising a coating applying means, a drier, a rotating brush driven at high speed and having thickly set relatively fine filaments,

a supporting cylinder for the paper while acted upon by said brush, and a calender 10 acting upon the paper successively in the order named.

In witness whereof I have hereunto set my hand.

ALEXANDER G. GILMAN.